

March 4, 1969

E. D. CRANE ET AL

3,430,569

SMOKE CARTRIDGE

Filed April 14, 1967



Fig. 1



Fig. 2



Fig. 3

INVENTORS:

EVERETT D. CRANE  
BURTON WERBEL

BY Harry M. Saragovitz,  
Edward J. Kelly, Herbert Berk  
& S. Dubroff ATTORNEYS

1

3,430,569

## SMOKE CARTRIDGE

Everett D. Crane, Dover, and Burton Werbel, West Orange, N.J., assignors to the United States of America as represented by the Secretary of the Army  
Filed Apr. 14, 1967, Ser. No. 631,106

U.S. Cl. 102—90  
Int. Cl. F42b 27/00

7 Claims

## ABSTRACT OF THE DISCLOSURE

A manually ignited, narrow column colored smoke marker having a metallic foil entirely encasing a smoke pellet and a portion of an igniting cord with the other portion of said cord extending outside of said foil. The smoke composition consists of a mixture of methylaminoanthraquinone, indanthrene, thiourea, potassium chlorate and a binder.

The invention relates to a smoke marker and more particularly to a manually ignited marker for producing a narrow column of colored smoke for signaling purposes.

In the past smoke assemblies were constructed by either pressing loose powder into a case, or by pressing or cementing a consolidated pellet into a case. With these assemblies, additional measures had to be taken to prevent the problem of flaming which has existed for many years in the art of producing smokes. Production of a colored cloud depends on an exothermal chemical reaction vaporizing a dye which has been mixed with the reactants. Subsequent condensation of the dye results in the colored cloud formation. Destruction of the dye may occur by the oxygen in the air reacting combustively with the hot dye vapors causing what is known in the art as flaming. Elimination of this flaming, other than through composition modification, has been attempted by one or more of the following methods used to build up pressure and to allow cooling of the dye vapor:

(a) Assembling into a container having one or more small openings.

(b) Keeping the surface of the composition at a distance from the openings, and

(c) In the instances of assemblies with center holes in composition, inhibiting the ends so that burning does not occur at the ends of the composition.

These methods are not always completely successful in the elimination of flaming, moreover, in the encasing of composition, difficulties are encountered such as:

(a) Shrinking of paper cases when consolidating loose powder therein, and

(b) Inadequate inhibition of the sides of pellets when cementing into the case.

The result of these methods was undesirable burning along the walls.

An advantage of the present invention is in its buoyancy. In instances where it becomes necessary to place a smoke signal in a water environment, the advantage of floating burning smoke cartridge will be apparent.

It is, therefore, an object of the present invention to provide a smoke cartridge that does not present the problem of flaming.

Another object is the provision of a smoke cartridge having superior cloud displays.

Still another object is to provide a smoke cartridge that is buoyant.

A further object is to provide a smoke cartridge having low size and weight for equivalent quantity of smoke composition.

The above objects as well as others together with the benefits and advantages of the invention will be ap-

2

parent upon reference to the detailed description set forth below, particularly when taken in conjunction with the drawings annexed hereto in which:

FIG. 1 shows a side view, partly broken away of the invention in the closed inoperative condition.

FIG. 2 shows an isometric view of the invention in the open operative condition.

FIG. 3 shows an exploded view of the invention.

As seen in the drawings the smoke cartridge 10 has an outer container 12 which is covered by a screw cap 14 having a polyethylene liner (not shown), this being done for protection against moisture in the atmosphere. Enclosed inside the container 12 is the pellet-foil-igniter cord assembly 16. The assembly 16 consists of a consolidated smoke pellet composition 18 wrapped in metal foil 20. On top of the composition 18 inside the foil 20 and extending therethrough is an igniter cord 22.

In the operation of the preferred assembly the igniter cord 22 is coiled on top of the composition 18 and the end of cord 22 emerges through the folds of the foil 20, which has been folded snugly around and against the composition 18. The length of igniter cord extending outside the foil wrapper is determined by safety considerations. For example, 2 3/4 inches (uncoiled) from initiating end to coil allows the operator from 3-6 seconds to move away. The number of coils inside the foil wrapper depends upon the composition used. The cord could also emerge through a hole cut into the foil.

As can be seen, no provisions for eliminating flame are required other than the foil wrap, which could be aluminum or the like, which allows a slight pressure buildup of insert gases formed by reaction, preventing oxygen in the atmosphere from diffusing in towards the reaction site. The dye vapors are cooled by contact with the metal foil before they reach the atmosphere.

In addition to the elimination of flaming attained by using the method of assembly of the invention disclosed herein, superior cloud displays are accomplished compared to those attained with equivalent weight and volume of smoke composition using prior methods. This superior performance is due to the burning that takes place on all surfaces of the smoke pellet, even though ignition starts at one surface, since the hot gases under the slight pressure developed, flow between the pellet and the foil to cause initiation on all surfaces. Even though the foil is wrapped around the pellet, the flexibility of the foil allows the gases to penetrate readily between the foil and pellet.

An example of composition yielding a red smoke is:

|                             | Percent |
|-----------------------------|---------|
| Methylaminoanthraquinone    | 44.5    |
| Indanthrene                 | 5.0     |
| Thiourea                    | 19.8    |
| Potassium chlorate          | 29.7    |
| Vinyl alcohol acetate resin | 1.0     |

The smoke cartridge is 1.2" in diameter and 0.9" in height. The cartridges are consolidated at 24,000 p.s.i. and wrapped in aluminum foil with two coils of igniter cord inside the foil in contact with the smoke composition. The total length of igniter cord used is 6 3/8", the uncoiled portion being 2 3/4 inches long. Therefore about 43% of the cord is outside and 57% inside the foil wrapper. The igniter cord used is of the safety fuze type for example, type PL thermalite, or the like.

The system consists of a match head and striker comparable to the existing smoke pot. Time of ignition is approximately six seconds. The heat required to ignite the smoke composition is 400° C. when pellets of composition are used and 200° C. when loose composition is used. The aluminum container consists of thin gage aluminum with each section threaded to form a water resistant con-

tainer. The compressed smoke pellet is wrapped in .001 in. thick aluminum foil.

The composition described above is used to provide a burning time of about fifteen seconds, but variations in percentage and particle size of some of the ingredients will yield different burning rates.

The composition can also be changed to provide for the use of different dyes when different colors are necessary.

We claim:

1. In a manually ignited smoke marker for producing 10 a narrow column of colored smoke for signalling purposes comprising:

a light weight container housing a compressed smoke composition and an igniter cord, said smoke composition consisting essentially of methylaminoanthraquinone, indanthrene, thiourea, potassium chlorate and a binder,

a metallic foil entirely encasing said composition and partially encasing said igniter cord, such that a portion of said cord is within said foil and the remaining portion is outside said foil, whereby upon the ignition of said cord, preliminary firing occurs outside of said foil wrapper and subsequent burning inside said foil wrapper causes the burning of said smoke composition throughout the entire surface thereof.

2. A smoke cartridge of the type described in claim 1 wherein said igniter cord extends through a cut in said metallic foil defining a small opening.

3. A smoke cartridge of the type described in claim 1 wherein an end of said igniter cord emerges through folds of said metallic foil which define a small opening.

4. A smoke cartridge of the type described in claim 1 wherein said container is waterproof.

5. A smoke cartridge of the type described in claim 1 wherein said smoke pellet composition consists essentially of 44.5% methylaminoanthraquinone, 5.0% indanthrene, 19.8% thiourea, 29.7% potassium chlorate and 1.0% vinyl alcohol acetate resin.

6. A smoke cartridge of the type described in claim 1 wherein said ignition cord is of the safety fuze type.

7. A smoke cartridge of the type described in claim 1 wherein said metallic foil is .001 inch thick.

#### References Cited

##### UNITED STATES PATENTS

|    |           |        |                     |        |
|----|-----------|--------|---------------------|--------|
| 15 | 1,448,073 | 3/1923 | Lucas et al. -----  | 102—90 |
|    | 1,918,594 | 7/1933 | Fladger -----       | 102—31 |
|    | 3,102,477 | 9/1963 | Stefan et al. ----- | 86—1   |
|    | 3,121,231 | 2/1964 | Reaves et al. ----- | 149—84 |
| 20 | 3,338,763 | 8/1967 | Kristal -----       | 149—84 |

##### OTHER REFERENCES

AMC Pamphlet, AMCP 706—187, Military Pyrotechnics Series, part three, properties of materials used in pyrotechnic compositions, Oct. 31, 1963 (herein referred to as M.P.S.), p. 150 required.

ROBERT F. STAHL, Primary Examiner.

U.S. Cl. X.R.

30 149—84; 252—359